

## UNITED STATES PATENT OFFICE

2,326,120

## METAL COATING COMPOSITION

George M. Black, Cleveland Heights, Ohio

No Drawing. Application March 21, 1940,  
Serial No. 325,187

12 Claims. (Cl. 106—219)

My invention relates to a composition of matter, and more particularly to a coating composition containing a chromium soap. My invention also relates to fabricated metallic articles, such as springs, and particularly to those of the ferrous base type in which the article is coated with a film containing a chromium soap and to the process of preparing such articles.

In applying paints or the usual coating compositions to metallic articles, such as those formed of a ferrous base metal, it is the practice to first thoroughly clean the metal. The cleaning is usually effected by treating the metallic article with an alkali, washing with hot water, and then treating with an acid. The article is then rinsed in cold water, dried, and the paint or composition is applied. When a fabricated article is to be coated, such as a ferrous base metal spring, it must be thoroughly cleaned before the paint or coating composition is applied, because in fabricating such articles it is necessary to utilize a mineral oil and unless the oil is first thoroughly removed, paints or other compositions which have heretofore been applied will not adhere to the metal surface.

One of the principal objects of my invention is to provide an improved composition of matter which may be applied to metallic articles, such as springs, without subjecting the article to the usual pretreating process and which when dried provides a durable film that will not chip or crack when subjected to expansion, percussion or contraction, and which is capable of preventing rust and corrosion of the base metal. The process of producing such springs may therefore be simplified and their production materially increased.

Another object is to provide an improved coating composition containing a chromium soap as a primary ingredient and which when dried is capable of producing a naturally black film having a hard, durable finish.

A further object is to provide an adherent coating composition containing a chromium soap and a solution or oil containing a mixture of resin and fatty acids.

Another object of my invention is to provide a metallic article, such as a spring, having a film thereon, one of the primary ingredients of which is a chromium soap.

A further object of my invention is to provide an improved process of applying a coating composition to metallic articles in which mineral oil is utilized during fabrication, such as springs, and which have a film of the mineral oil thereon.

A still further object of my invention is to pro-

vide an improved composition of matter comprising a chromium soap and an oil or solution containing resin and fatty acids, and a mineral oil.

In preparing my improved composition, I utilize 5 a chromium soap, such as chromium oleate, chromium stearate, chromium naphthenate, or a mixture of two or more of such soaps. Preferably, I utilize the chromium soap of an unsaturated fatty acid, such as chromium oleate. 10 Such soaps have corrosion resisting properties and expedite the drying of compositions in which they are present.

To provide a flowable material and to give 15 hardness, finish and adhesency to the final film, the chromium soap is dissolved in an oil or solution containing resin and fatty acids. To effect solution of the soap, it is necessary to mix the oil or solution with the soap and heat the mixture to a temperature varying from approximately 75° to 20 100° centigrade. The fatty acids in the oil or solution aid in dissolving the soap and preferably are higher fatty acids of the type which are present in or which may be derived from fats, vegetable oil or wood, such as pine. For instance, 25 fatty acids, such as palmitic, oleic, linoleic, or stearic acid, or mixtures thereof, are suitable. The resin acids are those which are found in the ordinary natural resins, or in resin oils, such as abietic acid, pimamic acid, and other resin acids, 30 the composition of which are not definitely known.

The resin and fatty acids may be present in the 35 oil or solution in widely varying proportions. The chromium soap, however, appears to be more soluble in the fatty acids than in the resin acids and consequently sufficient of the fatty acids should be present to provide a final composition having the desired amount of chromium soap. The resin acids on the other hand appear to 40 increase the hardness and enhance the finish of the final film. I do not desire, however, to be limited to any particular theory as to the function of the particular acids. Better results, however, have been obtained by utilizing a mixture of 45 resin and fatty acids than when only resin acids or fatty acids are employed.

An oil containing resin and fatty acids which is being sold commercially at the present time has proven very satisfactory for my purpose. 50 This oil is known commercially as rosin oil or tall oil and is obtained from pine wood in pulp forming processes. The composition of the oil varies widely, depending upon the source and type of pine wood which is utilized and contains resin acids in proportions varying from 12% to 58%.

fatty acids in proportions ranging from 18% to 83%, and from 5% to 24% of sterols. A semi-refined product is being sold under the trade name of "Liqro" which contains from 40% to 50% resin acids, 35% to 45% fatty acids, and 15% to 20% sterols, and a refined double distilled product is being sold under the trade name of "Indusol" which contains from 43% to 47% fatty acids, 38% to 42% of resin acids, and 13% to 17% sterols.

In preparing my improved composition, the chromium soap is dissolved in the solution or oil containing the resin and fatty acids, sufficient heat being utilized to effect solution. When tall oil is utilized as a solvent for the chromium soap, the composition is in the form of a thick paste and a thinner must be added to provide a coating composition. If it is desired to provide a film by drying in air, a volatile solvent, such as naphtha, may be utilized. When it is desired to bake the composition upon the surface to be coated, it is necessary to utilize a diluent which does not volatilize at ordinary temperatures, such as kerosene or mineral oil, or a combination thereof. The relative proportions of the chromium soap and the solution or oil containing the resin and fatty acids, may vary widely. For instance, in such a composition, the chromium soap may constitute from approximately 8% to 60% of the composition. Since the chromium soap, however, is the most effective corrosion preventing component of the coating composition, it is preferably present in considerably greater proportions than 8%, such as in amounts ranging from 20% to 35%.

While a composition may be provided which will dry in air, I preferably subject the coating to a baking operation to provide a more durable film. This is particularly true when it is applied to ferrous base articles, such as springs, which are subject to stresses in service.

To prevent too rapid drying during the baking operation, I preferably add a mineral oil in proportions sufficient to retard the drying to the extent necessary for the production of a smooth film. Mineral oil, however, has the tendency to separate from chromium soaps. When a resin oil or solution containing resin and fatty acids is present, however, this separation does not take place. In forming compositions containing mineral oil, it is therefore necessary to utilize a sufficient proportion of the oil or solution containing the resin and fatty acids to prevent separation of the chromium soap from the mineral oil. As the amount of mineral oil and chromium soap in the composition is varied, it is therefore necessary to vary the amount of oil containing the resin and fatty acids. In such compositions, the chromium soap may range from 8% to 60%, the oil containing the resin and fatty acids from 5% to 40%, and the mineral oil may be added in such proportions that a smooth film will be produced at the baking temperature, it being understood that as the quantity of mineral oil is increased beyond a predetermined amount, it is necessary either to increase the quantity of oil containing the resin and fatty acids or reduce the amount of chromium soap.

My improved composition may be applied to the article to be coated in any desired manner. For instance, it may be applied by brushing, dipping or spraying, the consistency being regulated for each process by the addition of the appropriate amount of thinner.

As previously stated, my improved composition

is especially adapted to be applied to fabricated articles, such as springs, because in fabricating such articles, a mineral oil is utilized which must be removed before the usual paint or coating

5 composition is applied. In ordinary processes, it is necessary to utilize phosphoric acid to remove the oil and consequently the present process of preparing such springs is not only time consuming but expensive. When my improved composition is employed, however, it may be applied to the springs without any preliminary treatment, because an oil or solution containing the resin and fatty acids is miscible with mineral oil and since the chromium soaps have a naturally dark 10 color, a dark coating is obtained without the addition of dyes or pigments.

The following specific example will serve to illustrate and explain my invention although it will be understood that I do not desire to limit 15 my invention to the specific procedure or the proportions specified.

A ferrous base metal spring, fabricated in the usual manner and having a film of mineral oil upon its surface, was coated with a composition 20 containing the following ingredients in approximately the proportions specified:

|                     | Per cent |
|---------------------|----------|
| Chromium oleate     | 10       |
| Mineral oil         | 20       |
| 30 Tall oil (Liqro) | 20       |
| Kerosene            | 48       |

The spring was dipped in the composition and then passed directly to a drying oven where it was subjected to a temperature of approximately 35 300° to 600° Fahrenheit for thirty minutes. An adherent durable film was provided which did not chip or crack when subjected to expansion, percussion, or contraction and which was effective in preventing rust and corrosion.

40 My improved composition may be utilized as the final coating or as a base coating over which may be applied ordinary paints, enamels or varnishes.

To those skilled in the art, many modifications of and widely differing embodiments and applications of my invention will suggest themselves without departing from the spirit and scope thereof. My disclosure and the description herein are purely illustrative and are not intended to be in any sense limiting.

What I claim is:

1. A composition of matter capable of adhering to a metal surface coated with a lubricant and of producing a hard durable film when applied to such surfaces and heated at a temperature of from 300° to 600° Fahrenheit and comprising from 8% to 60% of a chromium soap and a solvent for said soap including a mixture of resin acids and higher fatty acids in sufficient proportion to dissolve said soap, said fatty acids being of the type present in or derived from fats, vegetable oils and wood and said composition being free from inflammable ingredients 55 which are volatile at normal temperatures and from ingredients which cause a film formed from said composition at said temperature to chip or crack when subjected to expansion, contraction or percussion.

2. A composition of matter capable of adhering to metal surfaces coated with a lubricant and of producing a hard durable film when applied to such surfaces and heated at a temperature of from 300° to 600° Fahrenheit and comprising from 8% to 60% of a chromium soap

and a sufficient amount of a rosin oil composed predominantly of resin acids and higher fatty acids to dissolve said soap, the higher fatty acids being of the type present in or derived from fats, vegetable oils and wood and said composition being free from inflammable ingredients which are volatile at normal temperatures and from ingredients which cause a film formed from said composition at said temperature to chip or crack when subjected to expansion, contraction or percussion.

3. A composition of matter capable of adhering to metal surfaces coated with a lubricant and of producing a hard durable film when applied to such surfaces and heated at a temperature of from 300° to 600° Fahrenheit and comprising from 20% to 35% of a chromium soap and a sufficient amount of an oil composed predominantly of resin acids and higher fatty acids to dissolve said soap, said fatty acid being of the type present in or derived from vegetable oils, fats and wood and said composition being free from inflammable ingredients which are volatile at normal temperatures and from ingredients which cause a film formed from said composition at said temperature to chip or crack when subjected to expansion, contraction or percussion.

4. A coating composition capable of adhering to metal surfaces coated with a lubricant and of producing a hard durable film when applied to such surfaces and heated at a temperature of from 300° to 600° Fahrenheit and comprising from 20% to 35% of a chromium soap, a sufficient amount of tall oil to dissolve said soap and a diluent, said composition being free from inflammable ingredients which are volatile at normal temperatures and from ingredients which cause a film formed from said composition at said temperature to chip or crack when subjected to expansion, contraction or percussion.

5. A coating composition capable of adhering to metal surfaces coated with a lubricant and of producing a hard durable film when applied to such surfaces and heated at a temperature of from 300° to 600° Fahrenheit and comprising from 8% to 60% of a chromium soap, from 5% to 40% of an oil composed predominantly of resin acids and higher fatty acids, said fatty acids being of the type present in or derived from fats, vegetable oils and wood, and a sufficient amount of a diluent to provide a flowable composition, said composition being free from inflammable ingredients which are volatile at normal temperatures and from ingredients which cause a film formed from said composition to chip or crack when subjected to expansion, contraction or percussion.

6. A coating composition comprising at least 8% of a chromium soap, an oil composed predominantly of resin acids and higher fatty acids, the higher fatty acids being of the type which are present in or derived from fats, vegetable oils and wood, and a mineral oil which does not volatilize at normal temperatures, the mineral oil being present in sufficient proportion to retard the drying of the composition sufficiently to provide a smooth film when the composition is applied as a coating and subjected to heat and the oil containing resin and fatty acids being present in sufficient proportions to dissolve said soap and prevent separation of the chromium soap from the mineral oil.

7. A coating composition capable of adhering to metal surfaces coated with a lubricant and

of producing a hard durable film when applied to said surface and heated at a temperature of 300° to 600° Fahrenheit and comprising at least 8% of a chromium soap, 5% to 40% of tall oil, and a mineral oil which does not volatilize at normal temperatures in sufficient proportion to retard the drying of the composition sufficiently to provide a smooth film when the composition is applied and subjected to heat, said tall oil being present in sufficient proportion to prevent separation of the chromium soap from the mineral oil and said composition being free from inflammable ingredients which are volatile at normal temperatures and from ingredients which cause a film formed from said composition at said temperature to chip or crack when subjected to expansion, contraction or percussion.

8. A metallic article having a hard durable film thereon which does not chip or crack when subjected to expansion, contraction or percussion, said film consisting essentially of a chromium soap and the residual portion resulting from heating a mixture of resin acids and higher fatty acids to a temperature of 300° to 600° Fahrenheit in the presence of said soap for sufficient time to produce said film, said fatty acids being of the type present in or derived from fats, vegetable oil and wood and the residual portion of said resin and fatty acids being present in sufficient proportion to bind said chromium soap to the metallic article when heat is applied at said temperature.

9. A metallic spring formed of a ferrous base metal having a hard durable film thereon which does not chip or crack when subjected to expansion, contraction or percussion and consisting essentially of a chromium soap and the residual portion resulting from heating a mixture of resin acids and higher fatty acids at a temperature of 300° to 600° Fahrenheit in the presence of said soap for sufficient time to produce said film, the higher fatty acids being of the type present in or derived from fats, vegetable oils and wood and the residual portion of said resin and fatty acid being present in sufficient proportion to bind said soap to the metallic article when heat is applied at said temperature and said film being free from ingredients which chip or crack when subjected to expansion, contraction or percussion.

10. A ferrous base metal spring having a hard durable film thereon consisting essentially of a chromium soap and the residual portion resulting from heating mineral oil and a mixture of resin and higher fatty acids at a temperature of 300° to 600° Fahrenheit in the presence of said soap for sufficient time to produce said film, said fatty acids being of the type present in or derived from fats, vegetable oils and wood, and the residual portion of said mineral oil and said resin and fatty acids being present in sufficient proportion to bind said soap to the metallic article when heat is applied at said temperature, and said coating being free from ingredients which chip or crack when subjected to expansion, contraction or percussion.

11. A composition of matter capable of adhering to metal surfaces coated with a lubricant and of producing a hard durable film when applied to metal surfaces and heated at a temperature of 300° to 600° Fahrenheit and comprising from 8% to 60% of a chromium soap dissolved in tall oil, said composition being free from inflammable ingredients which are volatile at normal temperatures and from ingredients which are vola-

tile at normal temperatures and from ingredients which chip or crack when a film formed from said composition is subjected to expansion, contraction or percussion.

12. A metallic article having a hard durable film thereon, said film comprising from 8% to 60% of a chromium soap adherently united to

the metal by the residual portion of tall oil which has been heated at a temperature of 300° to 600° Fahrenheit in the presence of said soap for sufficient time to produce said film and being free from ingredients which chip or crack when subjected to expansion, contraction or percussion.

GEORGE M. BLACK.